

1

2,927,080

## CORROSION INHIBITOR

Roy A. Westlund, Jr., and Harry W. Rudel, Roselle, N.J., assignors to Esso Research and Engineering Company, a corporation of Delaware

No Drawing. Application August 6, 1956  
Serial No. 602,443

7 Claims. (Cl. 252—46.7)

This invention relates to corrosion inhibitors. Particularly, it relates to certain imidazolines which have been phospho-sulfurized to form compounds useful as corrosion inhibitors in normally liquid hydrocarbon compositions.

A serious problem in the operation of oil refining equipment, pipelines, storage tanks, etc. is the corrosion to the equipment caused by the petroleum crude oils, the various intermediate hydrocarbon fractions of the crudes, and even the finished petroleum products. Crude oils are generally acidic in nature and also contain sulfur compounds ranging from about 0.03% for Pennsylvania crudes to about 5.0% in Mexican crudes. Many of these various sulfur compounds break down into  $H_2S$  on heating in various stages of petroleum processing. The acidic materials and the  $H_2S$  are very corrosive to metal. Furthermore, crude oils and their various hydrocarbon fractions frequently contain a small amount of water which may have been initially present in the crude oil or which may have been added during various refining operations, such as steam stripping. The presence of water aggravates the corrosion problem, as water furnishes a medium for the acidic materials and sulfur compounds, thereby greatly increasing the degree of corrosivity. In general, the crude and various oil fractions at different stages of processing or storage may be considered as consisting of one or more of three phases; i.e., an oil phase, a water-oil phase, and a water phase. Of these three phases, encountered in refinery operations, the oil phase and the water-oil phase are the least corrosive and generally are easily inhibited. The water phase, on the other hand, which might be present in pipelines, storage or distilling operations, is a serious contributor to corrosion and is the most difficult to inhibit. A large number of various types of corrosion inhibitors have been proposed and are commercially available. However, it has been found that while most of these commercial inhibitors effectively inhibit rusting in the oil and water-oil phase, they have little effect on the water phase and, in fact, they frequently increase corrosion in the water phase.

It has now been found that certain imidazolines, which have been phospho-sulfurized, will form an additive which greatly reduces corrosion in refinery equipment caused by sulfur compounds, such as  $H_2S$  and various acidic materials. This additive may be added directly to the crude or to any of the normally liquid petroleum fractions at any stage of processing, or to the finished product. Generally, the lighter petroleum fractions exhibit a higher degree of corrosion and it may be desirable to add the inhibitor only to these lighter fractions after the original distillation of the crude into its various fractions. Generally, a concentration in the oily material of about 5 to 200 parts per million of inhibitor is effective in decreasing corrosion. However, the exact amount used will depend on the particular material or fraction to be inhibited, and will also depend on the particular crude oil which is being processed, as some types of crudes are

2

much more corrosive than others. Usually, about 10 to 100 p.p.m. of the inhibitor will be used. The additive material is left in the finished oil product and thereby furnishes protection against corrosion during the life of the product. The additive has no undesirable effect on the finished product and does not interfere with the addition of other additives to the final product.

The rust inhibitors of the invention are formed by reacting 1 mole of the imidazoline with from about 0.05 to 1.0 moles, e.g., 0.10 to 0.50 mole of a phosphorus sulfide compound; at temperatures of about 200 to 400° F., e.g., 300 to 350° F.; under an inert atmosphere to prevent oxidation, such as a nitrogen blanket; for from about 0.25 to 4.0 hours, e.g., 1.0 to 2.0 hours. After the reaction is completed, the reaction product is cooled to about 200 to 300° F., and may be filtered to give a final product which is useful as a corrosion inhibitor.

The imidazoline compounds useful in the invention are those having the general formula



wherein R is a straight or branched-chain alkyl or alkylene radical containing from about 2 to 22, e.g. 10 to 20, carbon atoms; and R<sub>1</sub> is a substituent selected from the group consisting of hydrogen and alkyl radicals of 1 to 6 carbon atoms. These imidazolines are readily prepared by reacting the proper organic acid with a suitable hydroxy substituted diamine. One such product which is commercially available under the name "Amine 220," is the reaction product of oleic acid and amino ethyl ethanolamine, said reaction product having the formula:



Another example of an imidazoline of the general formula is 1-hydroxy ethyl, 2-(heptadecadienyl-8,11)-2-imidazoline.

In carrying out the phospho-sulfurization, any of the various phospho-sulfurization agents may be used, such as  $P_2S_5$ ,  $P_4S_3$  and  $P_4S_7$ .

The invention will be more fully understood by the following examples:

## EXAMPLE I

0.667 mole of 1-hydroxy ethyl 2-(heptadecenyl-8) 2-imidazoline and 0.16 mole of  $P_2S_5$  were mixed at room temperature in a tall beaker. The mixture was heated under a nitrogen blanket to a temperature of about 300 to 310° F., while stirring. At this temperature, gas evolution began and the mixture was maintained at the 300 to 310° F. temperature for about 40 minutes, until said gas evolution ceased. The reaction mixture was then further heated to 350° F. and maintained at this temperature for about 45 minutes in order to complete the reaction. (The total heating time starting from room temperature was about 150 minutes.) The mixture was then cooled and filtered through filter paper at 300° F. and the product was further cooled to room temperature. The product was a dark greenish liquid, almost black.

The product of Example I was then tested for corrosion inhibiting properties in a test procedure designed to

simulate the operation of a pipestill, as described in the following example.

### EXAMPLE II

The corrosion rate tests were carried out in sealed Carius tubes which were about 19 mm. I.D. and about 70 cm. long. A mixture of 85 volume percent of a hydrocarbon fraction and 15 volume percent of water was placed in the tube, filling it to a level of about 42 cm. and providing an overhead vapor space of about 28 cm. The hydrocarbon fraction was a naphtha, commonly known as Stoddard Solvent, and having the following properties:

|                            |         |
|----------------------------|---------|
| 18 wt. percent aromatics   |         |
| 40 wt. percent naphthenes  |         |
| 42 wt. percent paraffins   |         |
| Boiling range, °F.         | 310-400 |
| Specific gravity 60/60 °F. | 0.790   |
| Flash point, °F.           | 107     |
| Aniline point, °F.         | 129     |

The tubes are placed in steel jackets and the jackets placed in an oil bath maintained at 140° C. for a period of 18 hours. The tube is immersed in the bath to a depth of 17 cm. so that boiling takes place in the lower part of the tube and condensation occurs in the upper part of the tube. This gives a three phase system consisting of:

- (1) Water phase—at the bottom of the tube.
- (2) Mixed hydrocarbon—water phase—in the center section of the tube.
- (3) Vapor phase—at the upper portion of the tube.

Weighed test coupons are placed in the appropriate phase and held by means of glass threads. In the water phase, the coupon is allowed to rest on the bottom of the tube. The coupons are prepared from a mild steel, of the type used in refinery equipment, and are cleaned by rinsing in acetone and then are grit-blasted to provide a fresh surface.

After placing the test specimens in position, the acidity of the medium was adjusted by the addition of HCl to a pH of 3, since it is known that pipestills operate under a pH of from about 2 to 6 or 7. Sufficient H<sub>2</sub>S was bubbled through the mixture until the concentration of H<sub>2</sub>S was about 50 p.p.m. (parts per million). A sufficient amount of the inhibitor to be evaluated was added to the mixture to provide an inhibitor concentration of 50 p.p.m. The tube is sealed and heated as described for 18 hours. After exposure, the tube is cooled and opened and the test specimens reweighed.

The percent protection is calculated from the following formula:

$$\text{Percent protection} = \frac{\text{loss of wt. by blank} - \text{loss of wt. of test specimen}}{\text{loss of wt. by blank}} \times 100$$

<sup>1</sup> The loss of wt. by the blank is determined by repeating the experiment with no inhibitor being present.

The above test was carried out on the product of Example I. For comparison purposes a number of other inhibitors, including several commercial inhibitors, were also tested by the above method.

The results showed that all the inhibitors tested gave excellent protection (better than 95%) in the mixed hydrocarbon-water phase. None of the inhibitors was effective in the vapor phase, due to the extremely low volatility of the inhibitors. In actual practice, protection of the vapor layer from "overhead" corrosion is effected by the use of volatile inhibitors such as ammonia or low molecular weight amines. These are well known inhibitors but due to their high volatility, they do not afford any protection to the lower layers, particularly the water phase. On the other hand, inhibition of the water phase is extremely difficult and it is with this phase that the

invention is particularly concerned. The usefulness of the compounds of this invention in reducing corrosion of the water phase is shown in the following table.

5 *Table 1.—Corrosion inhibiting properties of 50 p.p.m. of inhibitor in naphtha*

|    | Inhibitor                                                                                                                                                                                                                                                    | Percent Protection Water Layer |
|----|--------------------------------------------------------------------------------------------------------------------------------------------------------------------------------------------------------------------------------------------------------------|--------------------------------|
| 10 |                                                                                                                                                                                                                                                              |                                |
|    | H <sub>2</sub> N-(CH <sub>2</sub> -CH <sub>2</sub> -NH) <sub>3</sub> -CH <sub>2</sub> -OH-R-NH <sub>2</sub><br>C <sub>16</sub> H <sub>33</sub> -(NH-CH <sub>2</sub> -CH <sub>2</sub> ) <sub>3</sub> -NH <sub>2</sub>                                         | -3.5<br>-1.9                   |
| 15 | C <sub>16</sub> H <sub>33</sub> -(NH-CH <sub>2</sub> -CH <sub>2</sub> ) <sub>3</sub> -N-H-C <sub>16</sub> H <sub>33</sub>                                                                                                                                    | -52.0                          |
|    | H <sub>2</sub> N(CH <sub>2</sub> -CH <sub>2</sub> -NH) <sub>3</sub> -CH <sub>2</sub> -CH <sub>2</sub> -NH <sub>2</sub>                                                                                                                                       | -1.9                           |
|    | Polyrad 1110 <sup>1</sup>                                                                                                                                                                                                                                    | -156.0                         |
| 20 | H <sub>2</sub> N-(CH <sub>2</sub> -CH <sub>2</sub> ) <sub>3</sub> -N-(CH <sub>2</sub> -CH <sub>2</sub> ) <sub>3</sub> -N-(CH <sub>2</sub> -CH <sub>2</sub> ) <sub>3</sub> -N-R<br>(Where R=C <sub>6</sub> , C <sub>7</sub> , or C <sub>12</sub> alkyl group) | -152.0                         |
|    | Product of Example I <sup>2</sup>                                                                                                                                                                                                                            | 56.5                           |

<sup>1</sup> Commercial inhibitor which is the condensation product of rosin amine and ethylene oxide.

<sup>2</sup> Reaction product of P<sub>2</sub>S<sub>5</sub> and 1-hydroxyethyl, 2-heptadecenyl-8,2-imidazoline.

As seen from the above table, the product of the invention gave 56.5% protection in the water layer at 50 parts per million concentration. The other compounds tested, some of which are commercial inhibitors, actually increased corrosion in the water layer as indicated by the minus signs.

What is claimed is:

1. As a compound adapted to inhibit corrosion, the reaction product of 0.10 to 0.50 mole of a phosphorus sulfide and 1 mole of an imidazoline having the general formula:



45 wherein R is selected from the group consisting of alkyl and alkylene radicals containing from about 2 to 22 carbon atoms and R<sub>1</sub> is a substituent selected from the group consisting of hydrogen and alkyl radicals containing 1 to 6 carbon atoms, wherein said reaction is carried out at a temperature of about 200 to 400° F. for about 0.25 to 5.0 hours under an inert atmosphere.

50 2. As a corrosion inhibitor the reaction product of 0.05 to 1.0 mole of a phosphorus sulfide, and 1 mole of an imidazoline having the general formula:



65 wherein R is selected from the group consisting of alkyl and alkylene radicals containing from about 2 to 22 carbon atoms and R<sub>1</sub> is a substituent selected from the group consisting of hydrogen and alkyl radicals containing about 1 to 6 carbon atoms, said reaction being carried out at a temperature of about 200 to 400° F. for about 0.25 to 5.0 hours under an inert atmosphere.

70 75 3. As a corrosion inhibitor, the reaction product of

0.10 to 0.50 mole of a phosphorus sulfide and 1 mole of an imidazoline having the general formula:



wherein R is selected from the group consisting of alkyl and alkylene radicals containing about 10 to 20 carbon atoms and R<sub>1</sub> is a substituent selected from the group consisting of hydrogen and alkyl radicals containing 1 to 6 carbon atoms, said reaction being carried out at a temperature of about 300° F. to 350° F. for about 1.0 to 2.0 hours, under an inert atmosphere.

4. A petroleum hydrocarbon containing as a corrosion inhibitor, from about 5 to 200 parts per million of the reaction products of 0.05 to 1.0 mole of a phosphorus sulfide and 1 mole of an imidazoline having the general formula:



wherein R is selected from the group consisting of alkyl and alkylene radicals containing from about 2 to 22 carbon atoms and R<sub>1</sub> is a substituent selected from the group consisting of hydrogen and alkyl radicals containing 1 to 6 carbon atoms, wherein said reaction is carried out at a temperature of about 200 to 400° F. for about 0.25 to 5.0 hours under an inert atmosphere.

5. A method of inhibiting corrosion of steel in contact with a petroleum hydrocarbon fraction which comprises adding to said hydrocarbon fraction about 5 to 200 parts per million of a corrosion inhibitor which is the reaction product of 0.5 to 1.0 mole of a phosphorus sulfide and 1 mole of an imidazoline having the general formula:



wherein R is selected from the group consisting of alkyl and alkylene radicals containing from about 2 to 22 carbon atoms, and R<sub>1</sub> is a substituent selected from the group consisting of hydrogen and alkyl radicals containing 1 to 6 carbon atoms, wherein said reaction is carried

out at a temperature of about 200 to 400° F. for about 0.25 to 5.0 hours under an inert atmosphere.

6. A method of inhibiting corrosion of steel in contact with a petroleum hydrocarbon fraction containing a trace of water which comprises adding to said hydrocarbon fraction about 5 to 200 parts per million of a corrosion inhibitor which is the reaction product of 0.05 to 1.0 mole of a phosphorus sulfide, and 1 mole of an imidazoline having the general formula:



wherein R is selected from the group consisting of alkyl and alkylene radicals containing from about 2 to 22 carbon atoms and R<sub>1</sub> is a substituent selected from the group consisting of hydrogen and alkyl radicals containing 1 to 6 carbon atoms, said reaction being carried out at a temperature of about 200 to 400° F. for about 0.25 to 5.0 hours under an inert atmosphere.

7. A process for preparing a phosphorus sulfurized imidazoline which comprises reacting about 0.05 to 1.0 mole of a phosphorus sulfide per mole of imidazoline having the general formula:



wherein R is selected from the group consisting of alkyl and alkylene radicals containing from about 2 to 22 carbon atoms and R<sub>1</sub> is a substituent selected from the group consisting of hydrogen and alkyl radicals containing 1 to 6 carbon atoms, said reaction being carried out at a temperature of about 200 to 400° F. for a time of about 0.25 to 5.0 hours, under an inert atmosphere, and recovering a reaction product therefrom.

#### References Cited in the file of this patent

#### UNITED STATES PATENTS

|              |                     |               |
|--------------|---------------------|---------------|
| 2,382,775    | Cook et al. -----   | Aug. 14, 1945 |
| 50 2,539,424 | Hughes -----        | Jan. 30, 1951 |
| 2,542,981    | Bartleson -----     | Feb. 27, 1951 |
| 2,584,977    | Bartleson -----     | Feb. 12, 1952 |
| 2,592,497    | Waddey et al. ----- | Apr. 8, 1952  |
| 55 2,594,279 | Beare -----         | Apr. 29, 1952 |
| 2,614,075    | Bartleson -----     | Oct. 14, 1952 |
| 2,644,002    | Hoegberg -----      | June 30, 1953 |